

43321

## UNITED STATES PATENT OFFICE.

## SUBSTITUTE FOR MISSING XR

ISRAEL RABINOWICZ, OF SCHENECTADY, NEW YORK, ASSIGNOR OF TWO-  
THIRDS TO CHARLES STRATTMANN AND J. TELLER SCHOOLCRAFT, OF  
SAME PLACE.

## INSULATING COMPOUND.

SPECIFICATION forming part of Letters Patent No. 433,215, dated July 29, 1890.

Application filed March 29, 1890. Serial No. 345,861. (No specimens.)

*To all whom it may concern:*

Be it known that I, ISRAEL RABINOWICZ, a subject or citizen of the Russian Empire, residing at Schenectady, in the county of 5 Schenectady and State of New York, have invented certain new and useful Improvements in Insulating Compounds; and I do hereby declare the following to be a full, clear, and exact description of the invention, such as will enable others skilled in the art to which it appertains to make and use the same.

My invention or discovery has reference to a compound or mixture for fireproofing, waterproofing, and insulating purposes, a particular and preferred use of the composition being that of forming an insulating coating or envelope on wires used to conduct electric currents, the object of the invention being to provide a simple, cheap, efficient, readily-prepared, and quickly-applied compound for the purposes named; and to these ends the invention consists in the combination of the several ingredients or components, substantially as will be described and claimed.

25 In carrying my invention into practical effect I employ the following elements, constituents, or ingredients: first, palm stearine pitch; second, gilsonite; third, tartaric acid. This is the ordinary or dextro tartaric acid, having for its chemical formula  $C_4H_6O_6$  or  $CH(OH)-COOH$  or  $C'H(OH)-COOH$ . It is well known that tartaric acid when heated to 100° loses no water; when heated to 170° it fuses; but at a higher temperature it becomes carbonized, emitting during the process of carbonization a peculiar and highly-characteristic odor. These properties of tartaric acid make it valuable as an ingredient with my compound; fourth, some salt formed by the

40 tartaric acid, either that which it forms with potassium or sodium or antimony, or some other metal. The salt preferably employed is potassium bitartrate, which is one of the tartrates, and is an acid salt termed "hydric potassium tartrate" or "bitartrate of potassium," or the more usual term of "potassium bitartrate," its chemical formula being  $KH-C_4H_6O_6$ . Instead of using potassium bitartrate, the salts of other metals may be em-

ployed. These component parts are mixed together in suitable proportion to form the insulating, fireproofing, or waterproofing compound. They will be caused to readily unite by the application of heat. When warm and ready for insulating or other purposes, the compound will be in a liquid form and flexible, soft, pliant, or plastic; but when the compound is cooled it is quite hard, although still flexible. It has the general appearance of tar. It is generally applied to the article with which it is to be employed when in the warm or heated state. If it is to be used for the purpose of insulating an electric conducting-wire, it may be applied directly to the wire, forming a surrounding envelope or coating thereupon, or some substance—such as cotton, linen, or some textile fabric—may be saturated with the compound and then wound around or securely attached to the wire, thus providing the wire with an effective insulating material.

The salts of tartaric acid are incombustible absolutely. When subjected to a strong and powerful degree of heat, large quantities of water, steam, and carbonic acid are evolved therefrom. Therefore it will be seen that when my improved compound for fireproofing is used with any object for the purpose of rendering it non-combustible the effect will be, when fire or flame approaches the object to cause or form a bulb or bellows, and also to cause the carbonic acid, water, steam, and other elements to be given off by the compound, and they will act in a certain way to extinguish the flames in a measure, and, furthermore, there will be formed a hard non-combustible deposit of potassium carbonate which will effectually protect the object from becoming ignited by the flames.

It will now be proper to state the proportions in which the several ingredients of my compound are united. These proportions are as follows: I take seventy (70) pounds of palm stearine pitch, forty (40) pounds of gilsonite, nine (9) pounds of potassium bitartrate, and two (2) pounds of tartaric acid. These are then commingled and thoroughly mixed together. From this the proportion of the several ingredients will be fully understood.

It will be seen that I employ the inorganical salts of organical acids. This is an important feature of the invention, and it covers the combination of an inorganical with any organical acid.

Having thus described my invention, what I claim as new, and desire to secure by Letters Patent, is—

- 5 1. The herein-described compound for fire-proofing, waterproofing, insulating, and other purposes, which consists, essentially, of tartaric acid, gilsonite, a metallic salt, and pitch, substantially in the proportions specified.
- 10 2. The herein-described compound for fire-proofing, waterproofing, insulating, and other purposes, consisting, essentially, of tartaric acid, one of its salts, gilsonite, and palm stearine pitch, substantially in the proportions specified.
- 15 3. The herein-described compound for fire-

proofing, waterproofing, insulating, and other purposes, which consists, essentially, of tartaric acid, potassium bitartrate, gilsonite, and palm stearine pitch, substantially in the proportions specified.

4. The herein-described compound for fire-proofing and other purposes, which consists of tartaric acid, potassium bitartrate, gilsonite, and palm stearine pitch united in the following proportions: seventy (70) pounds of palm stearine pitch, forty (40) pounds of gilsonite, nine (9) pounds of potassium bitartrate, and two (2) pounds of tartaric acid.

In testimony whereof I affix my signature in presence of two witnesses.

ISRAEL RABINOWICZ.

Witnesses:

ALBERT L. HALSEY,  
FRANK H. SWART.